

[54] TEXTILE FINISH USING A COMBINATION  
OF AN AMINOPLAST RESIN AND  
MONOMETHYLOLDICYANDIAMIDE

[75] Inventor: Philip B. Roth, Somerville, N.J.

[73] Assignee: American Cyanamid Company,  
Stamford, Conn.

[22] Filed: July 2, 1973

[21] Appl. No.: 375,572

[52] U.S. Cl. .... 428/526; 427/390

[51] Int. Cl.<sup>2</sup> .... D06M 15/54; D06M 15/70

[58] Field of Search .... 117/139.4, 161 LN, 143 A;  
260/309.7, 551 C, 69 N, 849;  
427/390; 428/526

[56] References Cited

UNITED STATES PATENTS

2,247,353 7/1941 Auer ..... 117/139.4

|           |         |                      |             |
|-----------|---------|----------------------|-------------|
| 2,582,961 | 1/1952  | Burnell et al. ....  | 117/139.4 X |
| 2,662,071 | 12/1953 | Elod.....            | 117/139.4 X |
| 2,731,364 | 1/1956  | Reibnitz et al. .... | 117/139.4 X |
| 3,442,905 | 5/1969  | Herbes et al. ....   | 117/139.4 X |
| 3,488,701 | 1/1970  | Herbes et al. ....   | 117/139.4 X |
| 3,627,556 | 12/1971 | Roth et al. ....     | 117/139.4 X |

Primary Examiner—Michael R. Lusignan

Attorney, Agent, or Firm—H. G. Jackson

[57] ABSTRACT

The invention is a process for improving wrinkle recovery and durable press properties of cellulosic textile material while minimizing loss in resistance to abrasion and loss in tensile strength by applying to the material a combination of an aminoplast resin, monomethyloldicyandiamide, an accelerator and less than 4% acid and the material so treated.

12 Claims, No Drawings

TEXTILE FINISH USING A COMBINATION OF AN  
AMINOPLAST RESIN AND  
MONOMETHYLOLDICYANDIAMIDE

BACKGROUND OF THE INVENTION

1. Field of the Invention

The invention pertains to the art of improving wrinkle recovery and durable press properties by the use of a combination of certain organic chemicals.

2. Description of the Prior Art

In the textile finish field, cellulosic fabrics are treated with cross-linking reactants, for example, the aminoplast resins, to improve elasticity, i.e., wrinkle recovery, durable press properties, etc. However, the use of such treatment often is accompanied by a loss of strength and abrasion resistance. Various attempts have been made to overcome the undesirable loss of strength and abrasion resistance effects which accompany resin treatments. However, these attempts have been merely partially successful. In certain instances they depend on the use of less resin and thus the treated fabrics show poorer performance in desired characteristics. This invention is based on a process for improving textile finishes which involves the use of monomethyloldicyandiamide in combination with the normally used aminoplast resin finish whereby more desirable wrinkle recovery and durable press properties are achieved with greatly decreased loss of strength and abrasion resistance than is obtained when the aminoplast resin is applied in the absence of monomethyloldicyandiamide or when large amounts of phosphoric acid are used with the combination. U.S. Pat. No. 3,209,164; 3,079,279; 3,260,565 and 3,304,312 deal with ethyleneurea derivatives as wrinkle retardants or crease-proofing agents for textiles. The data in Table IV compares the crease-proofing properties of monomethyloldicyandiamide with other monofunctional agents. U.S. Pat. No. 2,582,961 teaches the use of monomethyloldicyandiamide and a resin with large amounts of phosphoric acid for flameproofing fabrics and improved crease and shrinkage resistance. Table V illustrates the improvement of my invention wherein the acid is reduced to less than 4% of the monofunctional reactant bath an improved tensile strength and flex abrasion are obtained.

SUMMARY OF THE INVENTION

The invention is a process for improving cellulosic textile material by imparting improved wrinkle recovery and durable press properties to the textile material accompanied by minimal loss of strength and abrasion resistance which comprises applying a combination of an aminoplast resin crosslinking agent, monomethyloldicyandiamide, an accelerator, and less than 4% acid to the material and the material so treated.

DESCRIPTION OF THE PREFERRED  
EMBODIMENTS

The invention is a process for improving textiles which involves the use of monomethyloldicyandiamide in combination with the normally used aminoplast resin finish and less than 4% acid whereby more desirable wrinkle recovery and durable press properties are achieved with greatly decreased loss of strength and abrasion resistance. Monomethyloldicyandiamide is a condensation product of equal molar amounts of form-

aldehyde and dicyandiamide. The synthesis is described in J. Prakt. Chemie, (2) Vol. 77 pg. 537 (1908).

The monomethyloldicyandiamide may be applied to the fabric either separately as a pretreatment followed by drying of the fabric before applying the aminoplast resin finish by a conventional method; or the monomethyloldicyandiamide may be applied simultaneously with aminoplast resin in the same bath. Thus, the combination is as effective in minimizing strength and abrasion loss when applied in the same bath as when applied as a pretreatment.

The normally encountered cross-linking agents identified as aminoplast resins may be used in the process. For example, as used herein the expression "aminoplast resin" includes many of the better known textile finishing resins classifiable as amino resins such as melamine formaldehyde condensates, guanamine formaldehyde condensates, triazole formaldehyde condensates, urea formaldehyde condensates, thiourea formaldehyde condensates, cyclic urea formaldehyde condensates, for example, 1,2-propylene urea formaldehyde condensates, 1,3-propylene urea formaldehyde condensates, and their corresponding thiourea derivatives and the alkylated, such as methylated, ethylated, and the like.

The following melamine formaldehyde resins are examples of resins useful in the process of my invention: tris(methoxymethyl) melamine, tris(methoxymethyl) dimethylol melamine, hexakis(methoxymethyl) melamine, bis(methoxymethyl) methylol melamine and the like. Examples of suitable guanamine formaldehyde condensates include the formaldehyde and alkylated formaldehyde condensates of methoxyacetoguanamine, propoxyacetoguanamide, butoxyacetoguanamine, lactoguanamine and others of the type known in the prior art and particularly those described in U.S. Pat. No. 2,887,409. Examples of urea and cyclic urea formaldehyde resins contemplated by the present invention are dimethylol urea, methylated methylol urea, methylated methylol thiourea, dimethylol 1,2-propylene urea, dimethylol ethylene urea, dimethylol ethylene thiourea, dimethylol 1,3-propylene urea, methylated dimethylol 1,3-propylene urea, and the like. Examples of triazole formaldehyde resins include dimethylol tetrahydro-5-ethyl-s-triazole-2, dimethylol tetrahydro-5-(2-hydroxyethyl)-s-triazole-2 and tetramethylethylene-5,5'-bis(tetrahydro-s-triazole-2).

As illustrative of the aminoplast resin useful in the process of the invention, examples are shown below with the results using (1) dimethyloldihydroxyethyleneurea, (2) 85% bis(methoxymethyl)uron; 15% hexakis(methoxymethyl)-melamine, (3) methylated hexamethylolmelamine with a crude urea component (uron), (4) polymethylolurea having 2.8 moles of combined formaldehyde. The preferred resin is dimethylol-dihydroxyethyleneurea.

The application of the reagents to the fabric is made under conventional conditions using also conventional accelerators, for example, a combination of 30% magnesium chloride and 2.5% aluminum chloride in water. In the process of the invention effective amounts of the monomethyloldicyandiamide range from about 4 to about 10% of the weight of the material for improving wrinkle resistance with minimal loss in textile strength and abrasion resistance, with a preferred range being about 6 to 8%. Effective amounts of the aminoplast resin for improving wrinkle resistance with minimal

loss in textile strength and abrasion resistance range from about 5 to about 35% of the weight of the material, with a preferred range being about 15 to 25%.

In the following examples which serve to illustrate the invention, the terms MMD and DMDHEU are used

but with the DMDHEU treatment omitted. All the fabric samples are then dried at 225°F. for two minutes, cured for one minute at 350° and finally tested for wrinkle recovery, strength and abrasion resistance. The data on these measurements are presented in Table I.

TABLE I

| Monofunctional Reactant                    | Crosslinking Reactant   | Wrinkle Recovery <sup>1</sup> | Tensile Strength <sup>2</sup><br>W×F | Abrasion Resistance <sup>3</sup><br>W×F |
|--------------------------------------------|-------------------------|-------------------------------|--------------------------------------|-----------------------------------------|
| none                                       | none                    | 199                           | 57 × 42                              | 370 × 311                               |
| 3% MMD+1.0% H <sub>3</sub> PO <sub>4</sub> | none                    | 209                           | 54 × 42                              | 331 × 343                               |
| none                                       | 15%                     | 269                           | 29 × 19                              | 93 × 101                                |
|                                            | DMDHEU+2.7% ACCELERATOR |                               |                                      |                                         |
| none                                       | 20%                     | 254                           | 26 × 17                              | 37 × 25                                 |
| none                                       | DMDHEU+3.6% ACCELERATOR |                               |                                      |                                         |
|                                            | 25%                     | 266                           | 25 × 16                              | 33 × 27                                 |
|                                            | DMDHEU+4.5% ACCELERATOR |                               |                                      |                                         |
| 5% MMD+1.6% H <sub>3</sub> PO <sub>4</sub> | 15%                     | 268                           | 39 × 25                              | 101 × 106                               |
| 5% MMD+1.6% H <sub>3</sub> PO <sub>4</sub> | DMDHEU+2.7% ACCELERATOR |                               |                                      |                                         |
|                                            | 20%                     | 276                           | 38 × 23                              | 114 × 80                                |
| 5% MMD+1.6% H <sub>3</sub> PO <sub>4</sub> | DMDHEU+3.6% ACCELERATOR |                               |                                      |                                         |
|                                            | 25%                     | 284                           | 39 × 24                              | 72 × 73                                 |
| 6% MMD+1.9% H <sub>3</sub> PO <sub>4</sub> | DMDHEU+4.5% ACCELERATOR |                               |                                      |                                         |
|                                            | 15%                     | 259                           | 38 × 26                              | 117 × 97                                |
| 6% MMD+1.9% H <sub>3</sub> PO <sub>4</sub> | DMDHEU+2.7% ACCELERATOR |                               |                                      |                                         |
|                                            | 20%                     | 279                           | 38 × 24                              | 91 × 70                                 |
| 6% MMD+1.9% H <sub>3</sub> PO <sub>4</sub> | DMDHEU+3.6% ACCELERATOR |                               |                                      |                                         |
|                                            | 25%                     | 267                           | 37 × 21                              | 85 × 100                                |
| 7% MMD+2.2% H <sub>3</sub> PO <sub>4</sub> | DMDHEU+4.5% ACCELERATOR |                               |                                      |                                         |
|                                            | 15%                     | 246                           | 41 × 25                              | 142 × 180                               |
| 7% MMD+2.2% H <sub>3</sub> PO <sub>4</sub> | DMDHEU+2.7% ACCELERATOR |                               |                                      |                                         |
|                                            | 20%                     | 275                           | 39 × 27                              | 141 × 168                               |
| 7% MMD+2.2% H <sub>3</sub> PO <sub>4</sub> | DMDHEU+3.6% ACCELERATOR |                               |                                      |                                         |
|                                            | 25%                     | 257                           | 41 × 26                              | 142 × 187                               |
| 8% MMD2.6% H <sub>3</sub> PO <sub>4</sub>  | DMDHEU+4.5% ACCELERATOR |                               |                                      |                                         |
|                                            | 15%                     | 245                           | 40 × 29                              | 147 × 147                               |
| 8% MMD2.6% H <sub>3</sub> PO <sub>4</sub>  | DMDHEU+2.7% ACCELERATOR |                               |                                      |                                         |
|                                            | 20%                     | 256                           | 43 × 28                              | 138 × 157                               |
| 8% MMD2.6% H <sub>3</sub> PO <sub>4</sub>  | DMDHEU+3.6% ACCELERATOR |                               |                                      |                                         |
|                                            | 25%                     | 249                           | 44 × 26                              | 113 × 107                               |

DMDHEU+4.5% ACCELERATOR

<sup>1</sup>W + F Total in Degrees<sup>2</sup>Measured in Pounds<sup>3</sup>Measured in Cycles.

for convenience to designate monomethyloldicyandamide and dimethyloldihydroxyethyleneurea, respectively. Standard test methods are used for evaluation. Wrinkle recovery measurements are made according to AATCC (American Assoc. of Textile Chemists and Colorists) Test Method 66-1968, tensile strength measurements according to ASTM (American Society of Testing Materials) Test Method D-1682-64 and abrasion resistance measurements according to ASTM Test Method D-1175-68.

## EXAMPLE 1

Application of MMD Monofunctional Reactant and DMDHEU Crosslinking Agent from Separate Baths

A. Three pad baths containing 15, 20 and 25 percent DMDHEU and 2.7, 3.6 and 4.5 percent accelerator\*, respectively, are prepared.

\*Accelerator is aqueous solution containing 30% magnesium chloride and 2.5% aluminum chloride.

B. Five pad baths containing 3, 5, 6, 7 and 8 percent MMD and 1.0, 1.6, 1.9, 2.2 and 2.6 percent phosphoric acid (85%), respectively, are prepared.

Each of the latter four MMD baths is applied by standard padding procedure to three samples each of 80 × 80 cotton percale (12 samples total) with a wet pickup of 80% on the weight of the fabric and the treated fabrics then dried. These treated samples along with samples in which the MMD treatment is omitted are then padded with DMDHEU baths of A above to a wet pickup of 80% on the weight of the fabric. The first pad bath (3% MMD) is similarly applied to cotton percale

The results in Table I illustrate that treatment with MMD alone makes no significant difference in wrinkle recovery, strength or abrasion resistance. DMDHEU alone can cause about 90% loss in abrasion resistance and about 60% loss in tensile strength while giving improvement in wrinkle recovery. The results in Table I further illustrate improvement in tensile strength and abrasion resistance with little or no decrease (sometimes an increase) in wrinkle recovery properties when cotton textile is treated with DMDHEU after pretreatment with MMD. Thus, application of 7% MMD and then 20% DMDHEU, compared to 20% DMDHEU and no MMD imparts an increase in wrinkle recovery from 254-275, an increase in strength from 26 × 17 to 39 × 27 and an increase in abrasion resistance from 37 × 25 to 141 × 168.

## EXAMPLE 2

Application of MMD Monofunctional Reactant Simultaneously with DMDHEU Crosslinking Agent

An aqueous pad bath containing 20% DMDHEU and 3.6% accelerator\* is prepared and divided into five portions. The first portion is used with no further modification. To the remaining four portions is added MMD to concentrations of 5, 6, 7 and 8% and phosphoric acid (85%) to concentrations of 1.6, 1.9, 2.2 and 2.6 percent respectively. Each of the five resin baths is applied by standard padding procedure to 80 × 80 cotton percale with wet pick up of 80% on the weight of the fabric. The treated samples are dried for two minutes at 225°F., cured for one minute at 350°F., and then tested

for wrinkle recovery, strength and abrasion resistance. The data on these measurements are presented in Table II.

\* Accelerator is aqueous solution containing 30% magnesium chloride and 2.5% aluminum chloride.

centration of 3.6%. One portion of each is used with no modification; to another portion of each is added MMD to a concentration of 7% and phosphoric acid (85%) to a concentration of 2.2%; to a third portion of

TABLE II

MMD Monofunctional Reactant and DMDHEU Crosslinking Agent Applied Simultaneously From Common Bath.

| Monofunctional Reactant                   | Crosslinking Reactant      | Wrinkle Recovery <sup>1</sup> | Tensile Strength <sup>2</sup> WxF | Abrasion Resistance <sup>3</sup> WxF |
|-------------------------------------------|----------------------------|-------------------------------|-----------------------------------|--------------------------------------|
| none                                      | 20% DMDHEU+3.6%ACCELERATOR | 303                           | 23 x 16                           | 35 x 47                              |
| 5% MMD+1.6%H <sub>3</sub> PO <sub>4</sub> | 20% DMDHEU+3.6%ACCELERATOR | 299                           | 33 x 23                           | 80 x 151                             |
| 6% MMD+1.9%H <sub>3</sub> PO <sub>4</sub> | 20% DMDHEU+3.6%ACCELERATOR | 299                           | 37 x 24                           | 108 x 119                            |
| 7% MMD+2.2%H <sub>3</sub> PO <sub>4</sub> | 20% DMDHEU+3.6%ACCELERATOR | 295                           | 40 x 27                           | 102 x 113                            |
| 8% MMD+2.6%H <sub>3</sub> PO <sub>4</sub> | 20% DMDHEU+3.6%ACCELERATOR | 288                           | 39 x 27                           | 115 x 171                            |

DMDHEU+3.6%ACCELERATOR

<sup>1</sup>W+F Total In Degrees

<sup>2</sup>Measured In Pounds

<sup>3</sup>Measured in Cycles

The results in Table II illustrate that the monofunctional reactant, MMD, is essentially as effective in minimizing tensile strength loss and abrasion resistance loss when applied simultaneously with the crosslinking reactant as when applied as a pretreatment (as in Example 1).

### EXAMPLE 3

#### Application of MMD Monofunctional Reactant with Miscellaneous Crosslinking Reactants

Solutions containing 20% of each of the following crosslinking reagents are prepared: bis(methoxymethyl)-uron + hexakis(methoxymethyl)melamine (85:15), methylated hexamethylolmelamine + crude uron component (75:25) and polymethylolurea containing 2.8 moles of combined formaldehyde (46-48% solids). To each of these is added accelerator\* to a con-

30 each of the original solutions is added MMD to a concentration of 8% and phosphoric acid (85%) to a concentration of 2.6%.

Each of these nine baths is applied by standard padding procedure to 80 x 80 cotton percale with a wet pick-up of 80% on the weight of the fabric. The treated fabrics are dried for two minutes at 225°F., cured for one minute at 350°F., and then tested for wrinkle recovery and loss in tensile strength and abrasion resistance. The data on these measurements are presented in Table III.

TABLE III

| Monofunctional Reactant                                  | Crosslinking Reactant                                                                                          | Wrinkle Recovery <sup>1</sup> | Tensile Strength <sup>2</sup> WxF | Abrasion Resistance <sup>3</sup> WxF |
|----------------------------------------------------------|----------------------------------------------------------------------------------------------------------------|-------------------------------|-----------------------------------|--------------------------------------|
| none                                                     | 20% solution of bis(methoxymethyl)uron+hexakis(methoxymethyl)melamine(85:15)+3.6% accelerator                  | 284                           | 19 x 17                           | 52 x 59                              |
| Solution of 7% MMD + 2.2% H <sub>3</sub> PO <sub>4</sub> | 20% solution of bis(methoxymethyl)uron+hexakis(methoxymethyl)melamine(85:15)+3.6% accelerator                  | 275                           | 41 x 27                           | 174 x 213                            |
| Solution of 8% MMD + 2.6% H <sub>3</sub> PO <sub>4</sub> | 20% solution of bis(methoxymethyl)uron+hexakis(methoxymethyl)melamine(85:15)+3.6% accelerator                  | 267                           | 42 x 27                           | 172 x 204                            |
| none                                                     | 20% solution of methylated hexamethylol melamine + crude uron component (75:25) +3.6% accelerator              | 299                           | 29 x 20                           | 93 x 81                              |
| Solution of 7% MMD + 2.2% H <sub>3</sub> PO <sub>4</sub> | 20% solution of methylated hexamethylol melamine + crude uron component (75:25) 3.6% accelerator               | 285                           | 40 x 27                           | 214 x 202                            |
| Solution of 8% MMD + 2.6% H <sub>3</sub> PO <sub>4</sub> | 20% Solution of methylated hexamethylol melamine + crude uron component (75:25) + 3.6% Accelerator             | 281                           | 42 x 26                           | 167 x 211                            |
| none                                                     | 20% Solution of polymethylolurea containing 2.8 moles combined formaldehyde (46-48% solids) + 3.6% Accelerator | 291                           | 26 x 28                           | 36 x 44                              |
| Solution of 7% MMD + 2.2% H <sub>3</sub> PO <sub>4</sub> | 20% Solution of polymethylolurea containing 2.8 moles combined formaldehyde (46-48% solids) + 3.6% Accelerator | 275                           | 41 x 27                           | 214 x 196                            |

TABLE III-continued

| Monofunctional Reactant                                  | Crosslinking Reactant                                                                                          | Wrinkle Recovery <sup>1</sup> | Tensile Strength <sup>2</sup> WxF | Abrasion Resistance <sup>3</sup> WxF |
|----------------------------------------------------------|----------------------------------------------------------------------------------------------------------------|-------------------------------|-----------------------------------|--------------------------------------|
| Solution of 8% MMD + 2.6% H <sub>3</sub> PO <sub>4</sub> | 20% Solution of polymethylolurea containing 2.8 moles combined formaldehyde (46-48% solids) + 3.6% Accelerator | 272                           | 39 x 27                           | 149 x 169                            |

\* Accelerator is aqueous solution containing 30% magnesium chloride and 2.5% aluminum chloride.

The results in Table III illustrate that when DMDHEU is replaced by other suitable crosslinking agents, the effect of the MMD monofunctional reactant on wrinkle recovery, abrasion resistance and tensile strength remains essentially the same.

The use of MMD is unique in its effect on fabric compared to other well known monofunctional agents. Table IV illustrates the use of monomethylol acrylamide (MMA) and monomethylol hydroxyethyl carbamate (MMD) as the monofunctional agent in place of MMD. The application of these agents with the aminoplast was similar to the application described in the examples above.

TABLE IV

| % MMA | % MMC | % DMDHEU | TENSILE STRENGTH |         | ABRASION RESISTANCE |
|-------|-------|----------|------------------|---------|---------------------|
|       |       |          | WRINKLE RECOVERY | WxF     | WxF                 |
| 5     | 0     | 0        | 201              | 55 x 46 | 462 x 524           |
| 5     | 0     | 20       | 294              | 23 x 17 | 35 x 35             |
| 6     | 0     | 0        | 190              | 58 x 41 | 369 x 557           |
| 6     | 0     | 20       | 289              | 23 x 16 | 39 x 44             |
| 7     | 0     | 0        | 188              | 58 x 45 | 362 x 500           |
| 7     | 0     | 20       | 288              | 24 x 18 | 41 x 41             |
| 8     | 0     | 0        | 173              | 59 x 43 | 338 x 565           |
| 8     | 0     | 20       | 298              | 25 x 17 | 41 x 56             |
| 0     | 5     | 0        | 184              | 53 x 43 | 420 x 470           |
| 0     | 5     | 20       | 292              | 24 x 16 | 48 x 41             |
| 0     | 6     | 0        | 185              | 56 x 42 | 374 x 526           |
| 0     | 6     | 20       | 294              | 24 x 18 | 37 x 44             |
| 0     | 7     | 0        | 175              | 56 x 44 | 325 x 583           |
| 0     | 7     | 20       | 296              | 27 x 17 | 39 x 69             |
| 0     | 8     | 0        | 174              | 55 x 43 | 409 x 581           |
| 0     | 8     | 20       | 297              | 29 x 14 | 61 x 75             |
| 0     | 0     | 0        | 195              | 58 x 45 | 410 x 623           |
| 0     | 0     | 20       | 286              | 24 x 17 | 38 x 47             |

It is readily seen from Table IV that MMA and MMC are not effective and cannot be used in place of MMD to achieve the same results.

#### EXAMPLE 4

An aqueous pad bath of 20% by weight of DMDHEU and 4% by weight of accelerator was divided into 11 equal portions. The first portion is used with no further modification. To the second portion is added 5% MMD and sufficient additional accelerator to raise the concentration of accelerator to 6%. The remaining nine portions are modified as follows:

25 A. Three pad baths containing 5, 6, and 7% MMD and 1.6, 1.9, and 2.2% phosphoric acid (85%), respectively, are prepared.

B. Three pad baths containing 5, 6, and 7% MMD and 1.34, 1.63 and 2.1% hydrochloric acid (37%), respectively, are preferred.

C. Three pad baths containing 5, 6, and 7% MMD and 0.9, 1.2, and 1.4% acetic acid (99%), respectively, are prepared.

35 Each of the pad baths are applied by standard padding procedure to samples of 80 x 80 cotton percale with a wet pickup of 90% on the weight of the fabric. The treated fabrics are then dried 1.5 minutes at 225°F., heated 1.0 minute at 350°F., and then tested for wrinkle recovery, tensile strength and abrasion resistance.

30 The results of this example presented in Table V, illustrate that without phosphoric acid, an even better improvement in tensile strength and flex abrasion is obtained. The use of hydrochloric or acetic acid in place 45 of phosphoric acid also produced similar improvements.

TABLE V

| Monofunctional Reactant                            | Crosslinking Reactant       | Application of MMD Monofunctional Reactant Together with DMDHEU Crosslinking Agent |                             |                                  |
|----------------------------------------------------|-----------------------------|------------------------------------------------------------------------------------|-----------------------------|----------------------------------|
|                                                    |                             | Wrinkle Recovery (Degrees WxF)                                                     | Tensile Strength (Lbs. WxF) | Abrasion Resistance (Cycles WxF) |
| None                                               | None                        | None                                                                               | 201                         | 53 x 43                          |
| None                                               | 20% DMDHEU + 4% Accelerator | 306                                                                                | 20 x 12                     | 38 x 26                          |
| 5% MMD                                             | 20% DMDHEU + 6% Accelerator | 284                                                                                | 36 x 27                     | 183 x 193                        |
| 5% MMD + 1.6% H <sub>3</sub> PO <sub>4</sub> (85%) | 20% DMDHEU + 4% Accelerator | 303                                                                                | 27 x 18                     | 80 x 66                          |
| 6% MMD + 1.9% H <sub>3</sub> PO <sub>4</sub> (85%) | 20% DMDHEU + 4% Accelerator | 300                                                                                | 29 x 20                     | 86 x 70                          |
| 7% MMD + 2.2% H <sub>3</sub> PO <sub>4</sub> (85%) | 20% DMDHEU + 4% Accelerator | 301                                                                                | 30 x 21                     | 108 x 94                         |
| 5% MMD + 1.34% HCl (37%)                           | 20% DMDHEU + 4% Accelerator | 292                                                                                | 32 x 21                     | 111 x 118                        |
| 6% MMD + 1.63% HCl (37%)                           | 20% DMDHEU + 4% Accelerator | 301                                                                                | 35 x 21                     | 114 x 128                        |
| 7% MMD + 2.1% HCl (37%)                            | 20% DMDHEU + 4% Accelerator | 289                                                                                | 33 x 22                     | 117 x 137                        |
| 5% MMD + 0.9% Acetic Acid (99%)                    | 20% DMDHEU + 4% Accelerator | 294                                                                                | 35 x 25                     | 156 x 183                        |
| 6% MMD + 1.2% Acetic Acid (99%)                    | 20% DMDHEU + 4% Accelerator | 284                                                                                | 37 x 27                     | 162 x 198                        |
| 7% MMD + 1.4% Acetic Acid (99%)                    | 20% DMDHEU + 4% Accelerator | 283                                                                                | 37 x 25                     | 187 x 193                        |

TABLE V-continued

| Monofunctional Reactant | Crosslinking Reactant | Wrinkle Recovery (Degrees WxF) | Tensile Strength (Lbs. WxF) | Abrasion Resistance (Cycles WxF) |
|-------------------------|-----------------------|--------------------------------|-----------------------------|----------------------------------|
| Acetic Acid (99%)       | Accelerator           |                                |                             |                                  |

1. Accelerator is aqueous solution containing 30% magnesium chloride and 2.5% aluminum chloride.

I claim:

1. A process for improving wrinkle resistance, with minimal loss in tensile strength and abrasion resistance, of cellulosic textile materials which comprises:

applying to the material an effective amount for improving wrinkle resistance with minimal loss in tensile strength and abrasion resistance of a tad bath of monomethyloldicyandiamide, aminoplast resin, a catalytic amount of an accelerator and less than 4% hydrochloric or acetic acid based on the weight of the tad bath and

heating the material to cure the composition to a water-insoluble state.

2. A process according to claim 1 wherein the aminoplast resin is dimethyloldihydroxyethyleneurea and the monomethyloldicyandiamide and resin are applied to the material from separate baths.

3. A process according to claim 2 wherein the monomethyloldicyandiamide is applied within a range of about 4 to about 10 percent of the weight of the material and the aminoplast resin is applied within a range of about 15 to about 25 percent of the weight of the material.

4. A process according to claim 1 wherein the aminoplast resin is dimethyloldihydroxyethyleneurea and the monomethyloldicyandiamide and resin are applied to the material simultaneously.

5. A process according to claim 4 wherein the monomethyloldicyandiamide is applied within a range of about 4 to about 10 percent of the weight of the material and the aminoplast resin is applied within a range of about 15 to about 25 percent of the weight of the material.

6. A process according to claim 1 wherein the aminoplast resin is dimethyloldihydroxyethyleneurea and the

monomethyloldicyandiamide and resin are applied to the material from separate baths and the acid is HCl.

7. A process according to claim 6 wherein the monomethyloldicyandiamide is applied within a range of about 4 to about 10 percent of the weight of the material and the aminoplast resin is applied within a range of about 15 to about 25 percent of the weight of the material.

8. A process according to claim 1 wherein the aminoplast resin is dimethyloldihydroxyethyleneurea and the monomethyloldicyandiamide and resin are applied to the material from separate baths and the acid is acetic acid.

9. A process according to claim 8 wherein the monomethyloldicyandiamide is applied within a range of about 4 to about 10 percent of the weight of the material and the aminoplast resin is applied within a range of about 15 to about 25 percent of the weight of the material.

10. Cellulose textile materials having improved wrinkle resistance and minimal loss in tensile strength and abrasion resistance cured with an effective amount for improving wrinkle resistance with minimal loss in tensile strength and abrasion resistance of monomethyloldicyandiamide, aminoplast textile resin, a catalytic amount of an accelerator and less than 4% hydrochloric or acetic acid based on the weight of the textile material.

11. Cellulosic textile materials according to claim 10 wherein the aminoplast resin is dimethyloldihydroxyethyleneurea and is within a range of about 15 to about 25 percent of the weight of the material and the monomethyloldicyandiamide is within a range of about 4 to about 10 percent of the weight of the material.

12. A process according to claim 1 wherein no acid is used in the bath.

\* \* \* \* \*